# EUROPEAN PATENT SPECIFICATION

(11) **EP 3 031 942 B1**
(45) Date of publication and mention of the grant of the patent: **12.07.2017**
(21) Application number: 14196949.3
(22) Date of filing: 09.12.2014
(51) Int. Cl.: C22C 38/00, C22C 38/22, C22C 38/24, C22C 38/44, C22C 38/46, C21D 1/18, C21D 1/25, C21D 8/02, C21D 9/02, C21D 9/52, C21D 1/56, C21D 1/55, C21D 6/00, F01D 25/00, F04B 39/10

(54) **Stainless steel strip for flapper valves**
Rostfreies Stahlband für Klappenventile
Bande d'acier inoxydable pour soupapes à clapet

(43) Date of publication of application: 15.06.2016
(73) Proprietor: voestalpine Precision Strip AB, 684 28 Munkfors (SE)
(72) Inventor: Millward, Chris, 667 31 Forshaga (SE); Nawaz, Azhar, 667 34 Forshaga (SE); Löf, Alexander, 652 20 Karlstad (SE)
(74) Representative: Johansson, Lars E.

(56) References cited:
- EP-A1- 1 739 199
- CN-A- 102 337 461
- JP-A- H0 533 244
- JP-A- H1 018 001
- JP-A- H1 018 002
- JP-A- H09 256 116
- JP-A- H10 110 248
- JP-A- 2009 203 528
- US-A- 5 714 114
- US-A1- 2009 301 615

## Description

### TECHNICAL FIELD

The invention relates to a stainless steel strip for flapper valves in compressors and other reed applications.

### BACKGROUND OF THE INVENTION

Flapper or reed valves are used in various types of applications where a specific type of compression cycle is regulated for a specific purpose. It can be a refrigeration cycle in a hermetic reciprocating compressor working uninterrupted in a refrigerator or in the air conditioner of a car. A flapper valve is basically a spring made from a pre-hardened steel strip. In its simplest form, the flapper valve is tongue shaped, where one end is fixed and the opposite end hangs free and regulates the liquid or gas flow in the compressor. The flapper valve suffers from both cyclic bending stresses and cyclic impact stresses during its service. Usually, these cyclic stresses eventually cause fatigue failure. Accordingly, the fatigue properties are of the utmost importance for the flapper valve material.

A flapper valve made of a steel strip of this invention has its fatigue properties optimized by a combined effect of modifications to the chemical composition of the steel, the non-metallic inclusions and the heat treatment.

Compressor OEMs require materials that have a higher fatigue life to improve the compressor's performance and life.

Furthermore, there is a growing interest in the industry to develop more energy efficient and quieter compressors. The coefficient of performance (COP) can be increased by increasing the valve lift and by reducing the thickness of the valves. Compressor designers therefore require valve materials that have enhanced damping properties in addition to fatigue strength improvement.

The existing steel grades used for reed valves are modified versions of a carbon steel AISI 1095 and a stainless steel AISI 420 produced via conventional melting, casting, rolling and heat treatment processes. However, the industry demands and resulting performance requirements mean that future flapper reeds will increasingly need to be made out of very thin steel strip with an increased fatigue life expectancy and higher damping properties.

US5714114 discloses a high hardness martensitic stainless steel with good pitting corrosion resistance, suitable for products which require both good corrosion resistance, particularly pitting corrosion resistance, and high hardness, such as nails, bolts, screws edged tools, springs and so on.

### DISCLOSURE OF THE INVENTION

The general object of the present invention is to provide a pre-hardened stainless steel strip for flapper valves having an optimized property profile such that it can be used to produce more efficient and reliable compressors.

A further object is to provide pre-hardened stainless steel strip for flapper valves, which reduces the flapper reed contribution to the overall noise levels of the compressor.

It is also an object of the present invention to provide a method of producing such an improved steel strip.

The foregoing objects, as well as additional advantages are achieved to a significant measure by providing a cold rolled and hardened martensitic stainless steel strip having a composition, microstructure and physical properties as set out in the claims.

The invention is defined in the claims.

### DETAILED DESCRIPTION

The importance of the separate elements and their interaction with each other as well as the limitations of the chemical ingredients of the claimed alloy are briefly explained in the following. All percentages for the chemical composition of the steel are given in weight % (wt. %) throughout the description. The amount of microstructural phases is given in volume % (vol. %). Upper and lower limits of the individual elements can be freely combined within the limits set out in the claims.

### Carbon (0.3 - 0.5 %)

is to be present in a minimum content of 0.3 %, preferably at least 0.32, 0.34, 0.36 or 0.36 %. Carbon is a strong austenite stabilizer with relatively large solubility in austenite. The upper limit for carbon is 0.5 % and may be set to 0.48, 0.46, 0.44 or 0.42 %. A referred range is 0.35 - 0.41 %. In any case, the amount of carbon should be controlled such that the amount of primary carbides of the type M₂₃C₆, M₇C₃ and M₆C in the steel is limited, preferably the steel is free from such primary carbides.

### Silicon (0.2 - 0.8 %)

Silicon is used for deoxidation. Si is a strong ferrite former and increases the carbon activity. Si is also a powerful solid-solution strengthening element and strengthens the steel matrix. This effect appears at a content of 0.2 %Si. A preferred range is 0.30 - 0.60 %.

### Manganese (0.2 - 1.0 %)

Manganese is an austenite stabilizer and contributes to improving the hardenability of the steel. Manganese shall therefore be present in a minimum content of 0.2 %, preferably at least 0.3, 0.35 or 0.4 %. When the content of Mn is too large the amount of retained austenite after finish annealing may be too high. The steel shall therefore contain maximum 1.0 % Mn, preferably maximum 0.8, 0.7 or 0.65 %.

### Chromium (12.0 - 15.0 %)

Chromium is a ferrite stabilizing element, which is added to impart corrosion resistance to the steel. Cr needs to be present in a content of at least 12.0 % in order to provide a passive film on the steel surface. The lower limit may be 12,4, 12, 6, 12, 8 or 13 %. When the content of Cr exceeds 15.0%, however, delta ferrite may form.

### Molybdenum (0.5 - 2.0 %)

Mo is a ferrite stabilizer and is known to have a very favourable effect on the hardenability. Molybdenum is essential for attaining a good secondary hardening response. The minimum content is 0.5 % and may be set to 0.6, 0.7 or 0.8 %. Molybdenum is strong carbide forming element and also a strong ferrite former. The maximum content of molybdenum is therefore 2.0 %. Preferably Mo is limited to 1.5, 1.3 or 1.1 %.

### Vanadium (0.01 - 0.20 %)

Vanadium forms evenly distributed fine precipitated carbides, nitrides and carbonitrides of the type V(N,C) in the matrix of the steel. This hard phase may also be denoted MX, wherein M is mainly V but other metals like Cr and Mo may be present to some extent. X is one or both of C and N. Vanadium shall therefore be present in an amount of 0.01 - 0.20%. The upper limit may be set to 0.1 or 0.08 %. The lower limit may be 0.02, 0.03, 0.04 or 0.05%.

### Nitrogen (0.02 - 0.15 %)

Nitrogen is a strong austenite former. N is restricted to 0.15% in order to obtain the desired type and amount of hard phases, in particular V(C,N). Higher nitrogen content may lead to work hardening, edge cracking and/or a high amount of retained austenite. When the nitrogen content is properly balanced against the vanadium content, vanadium rich carbonitrides V(C,N) will form. These will be partly dissolved during the austenitizing step and then precipitated during the tempering step as particles of nanometre size. The thermal stability of vanadium carbonitrides is considered to be better than that of vanadium carbides. Therefore the resistance against grain growth at high austenitizing temperatures is enhanced. The lower limit may be 0.02, 0.03, 0.04 or 0.05 %. The upper limit may be 0.12, 0.10, 0.08 or 0.06 %.

### Nickel (≤ 2.0 %)

Nickel is an austenite former. Ni may be present in an amount of ≤2.0 %. It gives the steel a good hardenability and toughness. However, because of the expense, the nickel content of the steel should be limited. The upper limit may therefore be set to 1.0, 0.5 or 0.5%. However, Ni is normally not deliberately added.

### Cobalt (≤ 2.0 %)

Cobalt is an austenite former. Co causes the solidus temperature to increase and therefore provides an opportunity to raises the hardening temperature. During austenitization it is therefore possible to dissolve larger fraction of carbides and thereby enhance the hardenability. Co also increases the Mₛ temperature. However, large amount of Co may result in a decreased toughness and wear resistance. The maximum amount is 2 % and may be set to 0.5 %. However, for practical reasons, such as scrap handling, a deliberate addition of Co is normally not made.

### Copper (≤ 2.0%)

Cu is an austenite stabilizing element but has a low solubility in ferrite. Cu may contribute to increasing the hardness and the corrosion resistance of the steel. However, it is not possible to extract copper from the steel once it has been added. This drastically makes the scrap handling more difficult. For this reason, the upper limit may be 1.0, 0.5, or 0.3 %. Copper is normally not deliberately added.

### Aluminium (≤ 0.06 %)

Aluminium may be used for deoxidation in combination with Si and Mn. The lower limit is set to 0.001, 0.003, 0.005 or 0.007% in order to ensure a good deoxidation. The upper limit is restricted to 0.06% for avoiding precipitation of undesired phases such as AlN and hard, brittle Alumina inclusions. The upper limit may be 0.05, 0.04, 0.03, 0.02 or 0.015%.

### Tungsten (≤ 2.0%)

In principle, molybdenum may be replaced by twice as much with tungsten because of their chemical similarities. However, tungsten is expensive and it also complicates the handling of scrap metal. The maximum amount is therefore limited to 2.0 %, preferably 0.5 % or 0.3 % and most preferably no deliberate additions are made.

### Niobium (≤ 0.05%)

Niobium is similar to vanadium in that it forms carbonitrides of the type M(N,C) and may in principle be used to replace part of the vanadium but that requires the double amount of niobium as compared to vanadium. However, Nb results in a more angular shape of the M(N,C) and these are also much more stable than V(C,N) and may therefore not be dissolved during austenitising. The maximum amount is therefore 0.05%, preferably 0.01 % and most preferably no deliberate additions are made.

### Ti, Zr and Ta (≤ 0.05% each)

These elements are carbide formers and may be present in the alloy in the claimed ranges for altering the composition of the hard phases. However, normally none of these elements are added.

### Boron (≤ 0.01%)

B may be used in order to further increase the hardness of the steel. The amount is limited to 0.01 %, preferably ≤ 0.005 or even ≤ 0.001 %.

### Ca and REM (Rare Earth Metals)

These elements may be added to the steel in the claimed amounts in order to further improve the hot workability and to modify the shape of non-metallic inclusions.

### Impurity elements

P, S and O are the main impurities, which have a negative effect on the mechanical properties of the steel strip. P may therefore be limited to 0.03%, preferably to 0.01%. S may be limited to 0.03, 0.01, 0.008, 0.0005 or 0.0002%. O may be limited to 0.003, 0.002 or 0.001%.

The present inventors have systematically investigated the effect of a modified chemical composition and a modified heat treatment on the mechanical properties of the flapper valve material. The modifications made to the chemical composition relative to the conventional material were mainly focused on increases in nitrogen and vanadium although some benefits were also gained from increases in austenite levels and tighter control over such elements as carbon, manganese and phosphorus.

The continuous hardening of valve strip was undertaken using different furnace parameters to map the hardening response of material from the conventional and modified chemical compositions. The production trials were carried out at a constant line speed with hardening temperatures in the range from 1000 °C to 1080°C, quenching into a molten lead alloy at a temperature in the range of 250°C to 350°C and tempering at temperatures in the range from 220°C to 600°C.

The mechanical properties resulting from these hardening trials on conventional material corresponded to:
- a yield strength Rp_{0.2} range between 1300 MPa and 1600 MPa,
- a tensile strength Rm range between 1740 MPa and 2100 MPa
- an elongation A50 range between 4 % and 6 %

Further continuous hardening trials were carried out on material with the modified chemical composition and non-metallic inclusion content. The production trials were carried out at a constant line speed with hardening temperatures in the range from 1050 °C to 1100°C, quenching into a molten lead alloy at a temperature in the range of 250°C to 350°C and tempering at temperatures in the range from 220°C to 600°C.

The mechanical properties resulting from further hardening trials on material with the modified chemical composition and non-metallic inclusion content corresponded to:
- a Rp_{0.2} range between 1400 MPa and 1750 MPa,
- a Rm range between 1970 MPa and 2300 MPa
- a A50 range between 4 % and 8 %

### EXAMPLE

In this example a stainless steel strip according to the invention is compared to a conventional stainless steel strip. The composition of the investigated steels was as follows:

| | **Conventional** | **Inventive** |
|---|---|---|
| C | 0.38 | 0.40 |
| Si | 0.36 | 0.42 |
| Mn | 0.48 | 0.56 |
| Cr | 13.1 | 13.4 |
| Mo | 0.98 | 0.99 |
| N | 0.017 | 0.052 |
| V | 0.009 | 0.055 |
| Ni | 0.31 | 0.15 |
| P | 0.018 | 0.018 |
| S | 0.0004 | 0.0006 |

Fe and impurities balance.

The cold rolled strips used for the hardening and tempering trials all had a thickness of 0.203 mm and a width of 140 mm. The strips were subjected to hardening and tempering in the above mentioned continuous hardening furnace. Tensile strength measurements were made according to ISO 6892:2009. Fig. 1 discloses tensile properties as a function of the austenitising temperature. Fig. 2 discloses the tensile properties as a function of the tempering temperature. The tensile strength (Rm) and the structure of the inventive steel is in accordance with claim 1.

### INDUSTRIAL APPLICABILITY

The inventive steel strip can be used for producing flapper valves for compressors having improved properties.

## Claims

1. A cold rolled and hardened martensitic/austenitic stainless steel strip for flapper valves in the compressors, wherein the steel strip
a) is made from steel consisting of in weight % (wt. %):
| | |
|---|---|
| C | 0.3 - 0.5 |
| Si | 0.2 - 0.8 |
| Mn | 0.2 - 1.0 |
| Cr | 12.0 - 15.0 |
| Mo | 0.5 - 2.0 |
| N | 0.02 - 0.15 |
| V | 0.01 - 0.20 |
| Ni | ≤ 2.0 |
| Co | ≤ 2.0 |
| Cu | ≤ 2.0 |
| W | ≤ 2.0 |
| Al | ≤ 0.06 |
| Ti | ≤ 0.05 |
| Zr | ≤ 0.05 |
| Nb | ≤ 0.05 |
| Ta | ≤ 0.05 |
| B | ≤ 0.01 |
| Ca | ≤ 0.009 |
| REM | ≤ 0.2 |
Fe and impurities balance,
b) has a matrix consisting of tempered martensite and between 5 and 15 volume % austenite,
c) has a tensile strength (Rₘ) of 1970-2300 MPa,
d) has a thickness of 0.07- 3 mm and a width of ≤ 500 mm.

2. A strip according to claim 1 fulfilling at least one of the following requirements:
| | |
|---|---|
| C | 0.35 - 0.41 |
| Si | 0.30 - 0.60 |
| Mn | 0.40 - 0.65 |
| Cr | 13 - 14 |
| Mo | 0.8 - 1.2 |
| N | 0.03 - 0.13 |
| V | 0.02 - 0.10 |
| Ni | ≤ 0.5 |
| Co | ≤ 0.5 |
| Cu | ≤ 0.5 |
| W | ≤ 0.5 |
| Al | ≤ 0.01 |
| Ti | ≤ 0.01 |
| Zr | ≤ 0.01 |
| Nb | ≤ 0.01 |
| Ta | ≤ 0.01 |
| B | ≤ 0.001 |
| Ca | 0.0005 - 0.002 |
and wherein the impurity contents of P, S and O fulfils the following requirements
| | |
|---|---|
| P | ≤ 0.03 |
| S | ≤ 0.03 |
| O | ≤ 0.003 |

3. A strip according to claim 1 or 2 fulfilling the following requirements:
| | |
|---|---|
| C | 0.35 - 0.41 |
| Si | 0.30 - 0.60 |
| Mn | 0.40 - 0.65 |
| Cr | 13 - 14 |
| Mo | 0.8 - 1.2 |
| N | 0.03 - 0.10 |
| V | 0.03 - 0.09 |

4. A strip according to any of the preceding claims, fulfilling at least one of the following requirements:
a tensile strength (Rₘ) of 2000-2200 MPa,
a yield strength (R_{P0.2}) of 1500-1750 MPa,
a Vickers Hardness (HV1) of 570 - 650,
a ductility A50 of 4-9 %.

5. A strip according to any of the preceding claims, fulfilling the following requirements:
reverse bending fatigue is > 850 MPa

6. A strip according to any of the preceding claims having a thickness of 0.1 - 1.5 mm and/or a width of 5 - 150 mm.

7. A strip according to any of the preceding claims, wherein the maximum globular inclusion size is 6 µm.

8. A strip according to any of the preceding claims, wherein the primary inclusion species are Silicate type with a maximum width of 4 µm.

9. A method of producing a strip according to any of claims 1-8, wherein the method comprises the following steps:
a) Hot rolling a steel having a composition as defined in any of claims 1-3,
b) Cold rolling the hot rolled strip to a thickness of 0.07-3mm,
c) Continuously hardening and tempering the cold rolled strip,
d) Optionally, slitting the cold rolled strip.

10. A method according claim 9, wherein the austenitising temperature is 1000 - 1150 °C in step c) and wherein tempering temperature is 200 - 600 °C.

11. A method according claim 9 or 10, wherein the hardening involves quenching the strip in a bath of molten lead or lead alloy, the bath preferably holding a temperature of 250 - 350 °C.

12. A method according to any of claims 9-11, wherein the steel used is produced by powder metallurgy and wherein the maximum globular inclusion size of said steel is 6 µm.

## Patentansprüche

1. Ein kaltgewalztes und gehärtetes martensitisches/ austenitisches, rostfreies Stahlband für Klappenventile in den Kompressoren, wobei das Stahlband
a) aus Stahl hergestellt ist, das aus folgendem in Gewichtsprozent (Gew.-%) besteht:
| | |
|---|---|
| C | 0,3 - 0,5 |
| Si | 0,2 - 0,8 |
| Mn | 0,2 - 1,0 |
| Cr | 12,0 - 15,0 |
| Mo | 0,5 - 2,0 |
| N | 0,02 - 0,15 |
| V | 0,01 - 0,20 |
| Ni | ≤ 2,0 |
| Co | ≤ 2,0 |
| Cu | ≤ 2,0 |
| W | ≤ 2,0 |
| Al | ≤ 0,06 |
| Ti | ≤ 0,05 |
| Zr | ≤ 0,05 |
| Nb | ≤ 0,05 |
| Ta | ≤ 0,05 |
| B | ≤ 0,01 |
| Ca | ≤ 0,009 |
| REM | ≤ 0,2 |
Fe und Verunreinigungen als Rest,
b) eine Matrix hat, die aus getempertem Martensit und zwischen 5 und 15 Gewichtsprozent Austenit besteht,
c) eine Zugfestigkeit (Rₘ) von 1970 - 2300 MPa hat,
d) eine Dicke von 0,07 - 3 mm und eine Breite von ≤ 500 mm hat.

2. Ein Band nach Anspruch 1, das mindestens eine der folgenden Voraussetzungen erfüllt:
| | |
|---|---|
| C | 0,35 - 0,41 |
| Si | 0,30 - 0,60 |
| Mn | 0,40 - 0,65 |
| Cr | 13 - 14 |
| Mo | 0,8 - 1,2 |
| N | 0,03 - 0,13 |
| V | 0,02 - 0,10 |
| Ni | ≤ 0,5 |
| Co | ≤ 0,5 |
| Cu | ≤ 0,5 |
| W | ≤ 0,5 |
| Al | ≤ 0,01 |
| Ti | ≤ 0,01 |
| Zr | ≤ 0,01 |
| Nb | ≤ 0,01 |
| Ta | ≤ 0,01 |
| B | ≤ 0,001 |
| Ca | ≤ 0,0005 - 0,002 |
und wobei der Gehalt an Verunreinigung von P, S und O die folgenden Voraussetzungen erfüllt
| | |
|---|---|
| P | ≤ 0,03 |
| S | ≤ 0,03 |
| O | ≤ 0,003 |

3. Ein Band nach Anspruch 1 oder 2, das folgende Voraussetzungen erfüllt:
| | |
|---|---|
| C | 0,35 - 0,41 |
| Si | 0,30 - 0,60 |
| Mn | 0,40 - 0,65 |
| Cr | 13 - 14 |
| Mo | 0,8 - 1,2 |
| N | 0,03 - 0,10 |
| V | 0,03 - 0,09 |

4. Ein Band nach einem der vorangegangenen Ansprüche, das mindestens eine der folgenden Voraussetzungen erfüllt:
eine Zugfestigkeit (Rₘ) von 2000 - 2200 MPa,
eine Dehngrenze (R_{P0,2}) von 1500 - 1750 MPa,
eine Vickers-Härte (HV1) von 570 - 650,
eine Formbarkeit A50 von 4 - 9 %.

5. Ein Band nach einem der vorangegangenen Ansprüche, das folgende Voraussetzungen erfüllt:
entgegengesetzte Biegedauerfestigkeit > 850 MPa

6. Ein Band nach einem der vorangegangenen Ansprüche, das eine Dicke von 0,1 - 1,5 mm und/oder eine Breite von 5 - 150 mm hat.

7. Ein Band nach einem der vorangegangenen Ansprüche, wobei die maximale kugelförmige Einschlussgröße 6 µm ist.

8. Ein Band nach einem der vorangegangenen Ansprüche, wobei die primäre Einschlussart Silikat-Typen mit einer maximalen Breite von 4 µm sind.

9. Ein Verfahren zur Herstellung eines Bands nach einem der Ansprüche 1 - 8, wobei das Verfahren die folgenden Schritte aufweist:
a) Warmwalzen des Stahls, das eine Zusammensetzung aufweist wie in einem der Ansprüche 1-3 definiert,
b) kaltwalzen des warmgewalzten Bands auf eine Dicke von 0,07 - 3 mm,
c) kontinuierliches Aushärten und Tempern des kaltgewalzten Bands,
d) wahlweise, das kaltgewalzte Band in Streifen schneiden.

10. Ein Verfahren nach Anspruch 9, wobei die Temperatur zur Austenitisierung in Schritt c) 1000 - 1150°C beträgt und wobei die Tempertemperatur 200 - 600°C ist.

11. Ein Verfahren nach Anspruch 9 oder 10, wobei beim Aushärten das Band in einem Bad, bestehend aus geschmolzenem Blei oder Bleilegierung, die vorzugsweise eine Temperatur von 250 - 350 °C aufweist, abgeschreckt wird.

12. Ein Verfahren nach einem der Anspruche 9 - 11, wobei der benutzte Stahl durch Pudermetallurgie hergestellt wird und wobei die maximale kugelförmige Einschlussgröße des vorbezeichneten Stahls 6 µm beträgt.

## Revendications

1. Bande d'acier inoxydable martensitique/austénitique, laminée à froid et durcie, pour soupapes à clapet dans des compresseurs, où ladite bande d'acier :
a) est fabriquée à partir d'un acier se composant en % en poids (% pds) :
| | |
|---|---|
| C | 0,3 - 0,5 |
| Si | 0,2 - 0,8 |
| Mn | 0,2 - 1,0 |
| Cr | 12,0 - 15,0 |
| Mo | 0,50 - 2,00 |
| N | 0,02 - 0,15 |
| V | 0,01 - 0,20 |
| Ni | ≤ 2,0 |
| Co | ≤ 2,0 |
| Cu | ≤ 2,0 |
| W | ≤ 2,0 |
| Al | ≤ 0,06 |
| Ti | ≤ 0,05 |
| Zr | ≤ 0,05 |
| Nb | ≤ 0,05 |
| Ta | ≤ 0,05 |
| B | ≤ 0,01 |
| Ca | ≤ 0,009 |
| REM | ≤ 0,2, |
le reste de Fe et d'impuretés,
b) possède une matrice se composant de martensite revenue et d'entre 5 et 15 % en volume d'austénite,
c) possède une résistance à la traction (Rₘ) de 1970 à 2300 MPa,
d) a une épaisseur de 0,07 à 3 mm et une largeur ≤ 500 mm.

2. Bande selon la revendication 1, répondant à au moins l'une des exigences suivantes :
| | |
|---|---|
| C | 0,35 - 0,41 |
| Si | 0,30 - 0,60 |
| Mn | 0,40 - 0,65 |
| Cr | 13 - 14 |
| Mo | 0,8 - 1,2 |
| N | 0,03 - 0,13 |
| V | 0,02 - 0,10 |
| Ni | ≤ 0,5 |
| Co | ≤ 0,5 |
| Cu | ≤ 0,5 |
| W | ≤ 0,5 |
| Al | ≤ 0,01 |
| Ti | ≤ 0,01 |
| Zr | ≤ 0,01 |
| Nb | ≤ 0,01 |
| Ta | ≤ 0,01 |
| B | ≤ 0,001 |
| Ca | 0,0005 - 0,002 |
et dans laquelle les teneurs en impuretés de P, S et O répondent aux exigences suivantes
| | |
|---|---|
| P | ≤ 0,03 |
| S | ≤ 0,03 |
| O | ≤ 0,003 |

3. Bande selon la revendication 1 ou 2, répondant aux exigences suivantes :
| | |
|---|---|
| C | 0,35 - 0,41 |
| Si | 0,30 - 0,60 |
| Mn | 0,40 - 0,65 |
| Cr | 13 - 14 |
| Mo | 0,8 - 1,2 |
| N | 0,03 - 0,10 |
| V | 0,03 - 0,09. |

4. Bande selon l'une quelconque des revendications précédentes, répondant au moins à l'une des exigences suivantes :
une résistance à la traction (Rₘ) de 2000 à 2200 MPa,
une limite d'élasticité de (R_{P0,2}) de 1500 à 1750 MPa,
une dureté de Vickers (HV1) de 570 à 650,
une ductilité A50 de 4 à 9 %.

5. Bande selon l'une quelconque des revendications précédentes, répondant aux exigences suivantes :
résistance aux efforts de flexion alternée > 850 MPa.

6. Bande selon l'une quelconque des revendications précédentes, ayant une épaisseur de 0,1 à 1,5 mm et/ou une largeur de 5 à 150 mm.

7. Bande selon l'une quelconque des revendications précédentes, dans laquelle la taille d'inclusion globulaire maximale est de 6 µm.

8. Bande selon l'une quelconque des revendications précédentes, dans laquelle les entités d'inclusion primaire sont de type silicate ayant une largeur maximale de 4 µm.

9. Procédé de production d'une bande selon l'une quelconque des revendications 1 à 8, où le procédé comprend les étapes suivantes :
a) laminage à chaud d'un acier ayant une composition telle que définie selon l'une quelconque des revendications 1 à 3,
b) laminage à froid de la bande laminée à chaud jusqu'à une épaisseur de 0,07 à 3 mm,
c) durcissement en continu et revenu de la bande laminée à froid,
d) éventuellement, refendage de la bande laminée à froid.

10. Procédé selon la revendication 9, dans lequel la température d'austénitisation est de 1 000 à 1 150°C à l'étape c) et dans lequel la température de revenu est de 200 à 600°C.

11. Procédé selon la revendication 9 ou 10, dans lequel le durcissement implique la trempe de la bande dans un bain de plomb fondu ou d'alliage de plomb fondu, le bain conservant de préférence une température de 250 à 350°C.

12. Procédé selon l'une quelconque des revendications 9 à 11, dans lequel l'acier utilisé est produit par métallurgie des poudres et dans lequel la taille d'inclusion globulaire maximale dudit acier est de 6 µm.
